

## UNITED STATES PATENT OFFICE

2,110,950

## MANUFACTURE OF STABLE PARAFFIN

Robert E. Burk and Herman P. Lankelma, Cleveland, Ohio, assignors to The Standard Oil Company, Cleveland, Ohio, a corporation of Ohio

No Drawing. Application February 10, 1936,  
Serial No. 63,278

4 Claims. (Cl. 87—19)

Paraffin as ordinarily refined, if subjected very much to heat deteriorates and becomes discolored. Particularly for example, where a paraffin bath has to be maintained in which the paraffin is heated as in the paraffining of paper and other articles to be water proofed etc., such difficulties are encountered. In accordance with the present invention however, it now becomes possible to prepare paraffin obviating such drawbacks.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The paraffin, obtained from any usual or desired source, as for instance paraffin-bearing petroleum oil, is decolorized, as by treatment with sulphuric acid, sulphur dioxide, etc., and while in molten condition there is incorporated a small amount of a tetrahydroxybicyclospiroindane, as for instance 3,3,3',3' tetramethyl 5,6,5',6' tetrahydroxybicyclospiroindane, etc. The amount of such treating agent is in general small. It need not exceed 1 per cent. Amounts of 0.001 to 0.5 per cent are satisfactory.

As an example: Paraffin in molten condition is treated by incorporation of 0.01 per cent of 3,3,3',3' tetramethyl 5,6,5',6' tetrahydroxybicyclospiroindane,



and the paraffin after thorough stirring, is cooled and solidified in cake or other desired form.

Other modes of applying the principle of the invention may be employed, change being made as regards the details described, provided the features stated in any of the following claims, or the equivalent of such, be employed.

We therefore particularly point out and distinctly claim as our invention:—

1. A process of preparing paraffin, comprising incorporating in the paraffin a small amount of an agent of the character of tetrahydroxybicyclospiroindane.

2. In a process of preparing paraffin, incorporating in the paraffin a small amount of 3,3,3',3' tetramethyl 5,6,5',6' tetrahydroxybicyclospiroindane.

3. Decolorized paraffin containing a small amount of an agent of the character of tetrahydroxybicyclospiroindane.

4. Decolorized paraffin containing a small amount of 3,3,3',3' tetramethyl 5,6,5',6' tetrahydroxybicyclospiroindane.

ROBERT E. BURK. 35  
HERMAN P. LANKELMA.